



US005254426A

**United States Patent [19]****Aslam et al.****Patent Number: 5,254,426****Date of Patent: Oct. 19, 1993****[54] METHOD OF MAKING A PROJECTION VIEWABLE TRANSPARENCY****[75] Inventors: Muhammed Aslam; Lawrence P. DeMejo, both of Rochester; Dinesh Tyagi, Fairport, all of N.Y.****[73] Assignee: Eastman Kodak Company, Rochester, N.Y.****[21] Appl. No.: 862,654****[22] Filed: Apr. 1, 1992****[51] Int. Cl.<sup>5</sup> G03G 13/01; G03G 13/20****[52] U.S. Cl. 430/124; 430/42; 430/99; 430/111****[58] Field of Search 430/45, 99, 111, 124, 430/42****[56] References Cited****U.S. PATENT DOCUMENTS**

- |           |         |               |           |
|-----------|---------|---------------|-----------|
| 3,578,797 | 5/1971  | Hodges        | 432/228 X |
| 4,791,447 | 12/1988 | Jacobs        | 430/124   |
| 4,913,991 | 4/1990  | Chiba et al.  | 430/45    |
| 4,931,618 | 6/1990  | Nagata et al. | 219/216   |
| 4,968,578 | 11/1990 | Light et al.  | 430/126   |
| 5,089,363 | 2/1992  | Rimai et al.  | 430/45    |
| 5,110,704 | 5/1992  | Inone et al.  | 430/110   |

5,126,221 6/1992 Chiba et al. 430/106 X

**FOREIGN PATENT DOCUMENTS**

88/300254 12/1988 Japan

*Primary Examiner*—Roland Martin*Attorney, Agent, or Firm*—Nixon, Hargrave, Devans & Doyle**[57] ABSTRACT**

A method of fusing an electrostatographic colored toner image on a transparent support to provide a projection viewable color transparency exhibiting excellent color clarity. The support comprises a polymer layer bearing the color toner image. The toner used to form the image has a loss tangent of 1.5 or less while the polymer that forms the layer bearing such image has a higher loss tangent. The transparent element is subjected to fusing in three distinct zones; a fusing zone where it is contacted with a fusing member, a cooling zone where contact with the fusing member is maintained and the toner image is cooled and a release zone where the toner image is released from the fusing member at a temperature where no toner image or polymer layer offset occurs.

**11 Claims, 1 Drawing Sheet**



FIG. 1



FIG. 2

**METHOD OF MAKING A PROJECTION  
VIEWABLE TRANSPARENCY**

**FIELD OF THE INVENTION**

This invention relates to a method of fusing an electrostatographic toner image on a transparent support comprising a polymer layer bearing such image. In one aspect, this invention pertains to such method for providing a projection viewable transparency wherein the unfused toner image and the polymer layer exhibit specific viscoelastic properties and the unfused toner image is converted to a fused image in three zones or stages while it is in contact with a fusing member. More particularly, this invention relates to such a fusing method for making a transparency capable of projecting an electrostatographic colored toner image exhibiting excellent color clarity.

**BACKGROUND**

In electrostatography an image comprising an electrostatic field pattern, usually of non-uniform strength, (also referred to as an electrostatic latent image) is formed on an insulative surface of an electrostatographic element by any of various methods. For example, the electrostatic latent image may be formed electrophotographically (i.e., by imagewise photo-induced dissipation of the strength of portions of an electrostatic field of uniform strength previously formed on a surface of an electrophotographic element comprising a photoconductive layer and an electrically conductive substrate), or it may be formed by dielectric recording (i.e., by direct electrical formation of an electrostatic field pattern on a surface of a dielectric material). Typically, the electrostatic latent image is then developed into an electrostatographic toner image by contacting the latent image with an electrostatographic developer containing an electrostatographic toner. If desired, the latent image can be transferred to another surface before such development. Although such techniques are typically used for black and white reproductions such as copying business correspondence, they are capable of forming a variety of single color or multicolor toner images.

A typical method of making a multicolor copy involves trichromatic color synthesis by subtractive color formation. In such synthesis successive latent electrostatic images are formed on a substrate, each representing a different color, and each image is developed with a toner of a different color and is transferred to a support (receiver). Typically, but not necessarily, the images will correspond to each of the three primary subtractive colors (cyan, magenta and yellow), and black as a fourth color, if desired. For example, light reflected from a color photograph to be copied can be passed through a filter before impinging on a charged photoconductive layer so that the latent electrostatic image on the photoconductive layer corresponds to the presence of yellow in the photograph. That latent image can be developed with a yellow toner and the developed image can be transferred to a support. Light reflected from the photograph can then be passed through another filter to form a latent electrostatic image on the photoconductive layer which corresponds to the presence of magenta in the photograph, and that latent image can then be developed with a magenta toner and

transferred to the same support. The process can be repeated for cyan (and black, if desired).

In the systems described previously herein, the toner images may be provided on a support such as paper, film, plastic or glass to which they are permanently fixed. A common technique for fixing such toner images to a support involves employing thermoplastic polymeric toner particles which include a colorant and fusing the particles to the support by the application of heat and pressure thereto. A suitable method involves passing the support with the toner particles thereon through a pair of opposed rolls, one a heated fuser roll and the other a non-heated or heated backup roll.

It is known to use the electrostatographic processes described, to provide transparencies that are primarily intended for viewing by transmitted light, for example, observing a projected image from an overhead projector. In a typical application the viewable fused toner image is either a single color or multicolor image but such viewable image may also have a single color portion and a multicolor portion. An acceptable transparency requires that the colored toner image exhibit good color clarity or chroma. Color clarity or chroma are terms used to describe the quality of an image projected by a transparency and high color clarity or high chroma refers to a faithful reproduction of the original colored image while low color clarity or low chroma refers to less than faithful or inaccurate reproduction of the original colored image. Low color clarity or chroma can result from light scattering or multiple reflections within a colored toner image which in turn results in a color shift upon projection of the color transparency and a failure to faithfully reproduce the colors of the original image. For example, bright yellow in an original image may appear as a muddy yellow.

It is also known that a transparency comprising a colored toner image exhibiting acceptable color clarity can be prepared in a fusing method where the image is pressure contacted with a highly polished heated roll. Such methods also provide toner images that have very high gloss since the toner image surface is smooth and highly reflecting. Unfortunately, toner images having such high gloss are not always desirable. For example, in a reflection color copy comprising a colored toner image it is often desirable to provide a toner image surface that has a low-level luster or fine matte appearance which has been found to be pleasing to a viewer. Such a surface has been achieved by contact fusing colored toner images using fusing surfaces that are textured, for example, textured fusing rolls. Unfortunately, the resultant textured toner image surfaces are known to deleteriously affect color clarity in a color transparency because they exhibit the harmful light scattering or multiple reflections described previously herein.

U.S. Pat. No. 4,791,447 issued Dec. 13, 1988, addresses the problem of providing glossy opaque toner images and high chroma transparencies using a fusing system comprising three roll members which cooperate to form a pair of roll nips.

In light of the previous discussion, it is obvious that it would be desirable to have a fusing method that is sufficiently flexible to provide transparencies comprising color toners having high color clarity and also be capable of providing toner images that exhibit a pleasing low-level luster of the type desired in certain reflection copy prints such as continuous tone reflection copy prints. This invention provides such a fusing method.

## SUMMARY OF THE INVENTION

In accordance with this invention, a transparency capable of projecting an electrostatographic colored toner image that exhibits excellent color clarity is obtained in a method which comprises (a) providing an element having a transparent support comprising a polymer layer bearing an image in colored toner particles that exhibit a loss tangent ( $\tan \delta$ ) up to about 1.5 upon fusing the image with heat and pressure, the polymer forming such layer having a loss tangent greater than the loss tangent of the toner, (b) passing the element successively through a fusing zone, a cooling zone and a release zone, (c) within the fusing zone, bringing the image and polymer layer into pressure contact with a surface of a fusing member at a temperature that fuses the image to the support and causes the polymer layer to flow, (d) maintaining contact between the fused image and the fusing member within the cooling zone while reducing the temperature of the fusing member, and (e) separating the fused image from the fusing member within the release zone at a temperature where the toner image and the polymer layer do not offset. The aforementioned loss tangent ( $\tan \delta$ ) values describe the rheological characteristics or viscoelasticity of a polymeric material, as will be discussed in greater detail hereinafter.

The method of this invention provides a technique for separating the contact fusing and fusing member release events that occur during the process by a substantial cooling phase. This is a significant distinction from roll fusing processes of the type employed in U.S. Pat. No. 4,791,447, referred to previously, where such events take place substantially simultaneously. Separating the contact fusing and fusing member release events according to the process of this invention makes it possible to use a fusing temperature which is sufficient to cause the toner particles and the polymer layer on the support to flow sufficiently to form a fused color toner image that exhibits high clarity and is adhesively adhered to the transparent support. The fused image and polymer layer can then be separated from the fusing member after cooling when they do not offset onto the fusing member. Accordingly, the process of this invention is easily controlled and represents an obvious advantage over roll fusing techniques of the type described in U.S. Pat. No. 4,791,447. Other advantages of this invention will be described or become obvious from the following description.

It should also be noted that Japanese laid-open Application Number 88/300,254, published Dec. 7, 1988 indicates that toners exhibiting high viscosity (elastic) flow, as indicated by loss tangent values of 1.30 to 1.60 can be expected to form fused toner images that have irregular non-glossy surfaces. Such surfaces do, of course, provide light-scattering and multiple reflections of the type referred to previously herein and would be expected to deleteriously affect the color clarity of a fused color toner image. Accordingly, it was quite unexpected that colored toners exhibiting even more viscous flow than those in the aforementioned Japanese laid-open Application, as indicated by loss tangent values of 1.5 or less, could be used in the method of this invention to provide projection viewable color transparencies having good color clarity.

## BRIEF DESCRIPTION OF DRAWINGS

FIG. 1 is a schematic illustration of apparatus suitable for carrying out the method of this invention.

FIG. 2 is a schematic illustration of other apparatus suitable for carrying out the method of this invention.

## DETAILED DESCRIPTION OF THE INVENTION

10 The unfixed or unfused colored toner image that is fused in the method of this invention can be generated using any electrostatographic image-forming process that forms a toner image comprising discrete toner Particles having the loss tangent up to 1.5 referred to previously herein. Such toner images can comprise line copy, 15 continuous tone images and half-tone images as well as combinations thereof. The toner images are conveniently generated using electrostatographic processes of the type described hereinbefore, including the toner images comprising single color images and multicolor images, for example, four-color images prepared using digital four-color, full-color printers. Suitable color toner images that can be fused in the method of this invention include the lower gloss colored toner images described in Japanese laid-open Application No. 88/300,254, published Dec. 7, 1988 which have loss tangent values up to 1.5.

FIG. 1 illustrates preferred apparatus suitable for fusing or fixing an electrostatographic colored toner image to provide a transparency having high color clarity according to the method of this invention. FIG. 1 depicts a fusing device 1 which comprises a heating roll 2, a roll 3 spaced from the heating roll 2, a fusing member which is trained about heating roll 2 and roll 3 35 as an endless or continuous web or belt 4 which is conveyed in a counterclockwise direction, as viewed in FIG. 1, upon rotation of the heating roll 2 and roll 3. Backup or pressure roll 5 is biased against the heating roll 2 and the continuous belt 4 is cooled by impinging air provided by blower 6 disposed above the belt 4. In operation, transparent support 7 comprising a polymer layer having a loss tangent greater than the unfused colored toner particles on its surface is transported in the direction of the arrow into the nip between heating roll 2 and backup or pressure roll 5 which can be heated if desired, where it enters a fusing zone extending about 40 2.5 cm laterally along continuous belt 4. Following fusing in the fusing zone, the fused image then continues along the path of belt 4 and into the cooling zone (about 45 5 to 25 cm in length) in the region following the nip between heating roll 2 and pressure roll 3. Upon exiting the fusing zone, belt 4 is cooled slightly upon separation from heating roll 3 and then additionally cooled in a controlled manner by air that is caused to impinge upon belt 4 by blower 6. The fused toner image on support 7 then exits the cooling zone and separates from belt 4 as the belt passes around roll 3 and is transported to copy collection means such as a tray (not shown). Support 7 bearing the fused image is separated from the fusing member within the release zone at a temperature where 50 no toner image or polymer layer offset occurs. Separation is expedited by using a roll 3 of relatively small diameter, e.g. a diameter of about 2.5 to 4 cm. After 55 passing through the three distinct zones, i.e. the fusing zone, cooling zone and release zone, the fused colored toner image exhibits high color clarity. The extent of each of the three zones and the duration of time the toner image resides in each zone can be conveniently 60 65

controlled simply by adjusting the velocity or speed of belt 4. The velocity of the belt in a specific situation will depend upon several variables, including, for example, the temperature of the belt in the fusing zone, the temperature of the cooling air and the composition of the colored toner particles. U.S. Pat. No. 3,931,618, issued Jun. 5, 1990, describes an image glazing device that is used to apply a gloss to a fused toner image or a dye image. Such device has several features in common with the fusing apparatus depicted in FIG. 1 which features are described in detail in the patent. Accordingly, U.S. Pat. No. 3,931,618 is hereby incorporated by reference herein.

FIG. 2 illustrates another device suitable for fusing an electrostatographic colored toner image on a transparent support to provide a projection viewable transparency having excellent color clarity. In this device the fusing member is a roll rather than the continuous web shown in FIG. 1. As shown in FIG. 2, the fusing device 9 comprises a roll 10, forming a nip with backup or pressure roll 11 and another nip with roll 12 and continuous conveyor means 17 trained partly about rolls 10 and 12, and scive 18. Roll 10 rotates in a counterclockwise direction while rolls 11 and 12 rotate in a clockwise direction, as viewed in FIG. 2. The surface of roll 10 is heated by radiant heat from a heater 13 and is cooled by air provided by blower 14. Transparent support 16 comprises a polymer layer which bears unfused colored toner image 15. In operation, support 16 bearing unfixed or unfused toner image 15 is conveyed in the direction of the arrow on continuous conveyor means 17 through the nip between rolls 10 and 11 around roll 10 and continues through the nip between rolls 10 and 12. The toner image passes through the fusing zone extending through the nip between rolls 10 and 11 and proceeds through the cooling zone where blower 14 impinges air upon conveyor 17 which cools support 16 bearing fused colored toner image and the surface of roll 10. Upon exiting the cooling zone support 16 bearing the fused colored toner image is separated by scive 18 from roll 10 (now in a cooled condition) after exiting the nip between roll 10 and roll 12. Upon separation support 16 bearing the fused colored toner image is transported by copy handling means to copy collection means such as a tray (not shown). The fused colored toner image is separated from the cooled surface of roll 10 at a temperature where no toner image or polymer layer offset occurs.

It is essential to this invention that the colored toner image fused in the inventive method comprise toner particles that exhibit a loss tangent which does not exceed about 1.5, typically about 0.5 to 1.5, and the polymer layer bearing such image have a loss tangent which is greater than that of the toner particles. As discussed in Japanese laid-open Application No. 88/300,254, referred to hereinbefore, and in U.S. Pat. No. 4,913,991, issued Apr. 3, 1990, loss tangent describes the rheological characteristics (viscoelasticity) of a toner and is the ratio of the loss modulus ( $G''$ ) to the storage modulus ( $G'$ ). This relationship can be described by the following equation:

$$\tan\delta = \frac{\text{loss modulus}(G'')}{\text{storage modulus}(G')}$$

The rheological characteristics of the toner particles and the polymer forming the surface of the support used in this invention from which such loss tangent can be determined can be measured using conventional equip-

ment, for example, a rheometer. An example of a suitable rheometer is a Rheometrics Model RDA 700 (commercially available from Rheometrics, Inc., Piscataway, N.J.) Another example is the Rheometrics Dynamic Spectrometer RDS-7700 made by Rheometrics, Inc., which is mentioned in Japanese laid-open Application Number 88/300,254 and U.S. Pat. No. 4,913,991. The rheological characteristics of the toners and layer-forming polymers used in this invention were measured with the Rheometrics Model RDA using parallel plates in a sinusoidal shear mode. Measurements were made at temperatures ranging from 100° to 250° C. and at frequencies ranging from 0.1 to 100 rad./sec. The loss tangent values referred to in this specification and claims were determined for a storage modulus ( $G'$ ) of 10 dynes/cm<sup>2</sup> and, therefore, can be directly compared to the loss tangent values reported in Japanese laid-open Application Number 88/300,254 and U.S. Pat. No. 4,913,991.

The aforementioned loss tangents are largely determined by the toner binder polymer or the layer-forming polymer which is the principle determinant of viscoelastic properties. As understood by those skilled in the art, and as illustrated by the following Examples, Japanese laid-open Application Number 88/300,254 and U.S. Pat. No. 4,913,991; the loss tangent of a given polymer material depends upon several variables, including polymer architecture (chain-branching, cross-linking or lack thereof) molecular weight distribution, glass transition temperature and additives. Accordingly, the toner particles are formulated with the type of polymer or combination of such polymers which meet the criteria needed to provide a desired loss tangent. Suitable toner polymer materials having the low loss tangent values can comprise an additive which adjusts the loss tangent of a polymer to less than 1.2. Such additives can be used in concentrations up to 50 weight percent of the toner polymer material, and include vinyl addition and/or polycondensation polymers that are high molecular weight and can be highly cross-linked. Such additive polymers frequently have  $T_g$  values in the range of about 65° to 125° C. Polymeric beads, e.g. polymethylmethacrylate beads can be employed as useful additives. Accordingly, the toner particles and layers bearing such particles are formulated with the type of polymer or combination of such polymers which meet the criteria need to provide a desired loss tangent. Suitable toner binder materials can comprise an additive which adjusts the loss tangent of a binder polymer to less than about 1.5. Such additives can be used in concentrations up to 50 weight percent of the toner binder material, and include vinyl addition and/or polycondensation polymers that are high molecular weight and can be highly cross-linked. Such additive polymers frequently have  $T_g$  values in the range of about 65° to 125° C. Polymeric beads, e.g. polymethylmethacrylate beads can be employed as useful additives. A wide variety of polymer materials can be employed in the colored toner and polymer layers bearing such toner, including vinyl addition polymers and condensation polymers. Such polymers are chosen for their loss tangent values as well as good combinations of advantageous properties, such as toughness, transparency, and adequate adhesion to substrates. Vinyl addition polymers that are useful can be linear, branched or lightly cross-linked. The most widely used condensation polymers are polyesters which are polymers in which backbone

recurring units are connected by ester linkages. Like the vinyl addition polymers, polyester useful as binder materials in toner particles and as layer-forming polymers can be linear, branched or lightly cross-linked. They can be fashioned from any of many different monomers, typically by polycondensation of monomers containing two or more carboxylic acid groups (or derivatives thereof, such as anhydride or ester groups) with monomers containing two or more hydroxy groups. Specific examples of useful binder polymers include olefin homopolymers and copolymers, such as polyethylene, polypropylene, polyisobutylene, and polyisopentylene; polyfluoroolefins such as polytetrafluoroethylene; polyhexamethylene adipamide, polyhexamethylene sebacamide and polycaprolactam; acrylic resins, such as polymethylmethacrylate, polyacrylonitrile, polymethylacrylate, polyethylmethacrylate and styrene-methymethacrylate or ethylene-methyl acrylate copolymers, ethylene-ethyl acrylate copolymers, ethylene-ethyl methacrylate copolymers, polystyrene and copolymers of styrene with unsaturated acrylic monomers of the type mentioned hereinbefore, cellulose derivatives, such as cellulose acetate, cellulose acetate butyrate, cellulose propionate, cellulose acetate propionate, and ethyl cellulose; polyvinyl resins such as polyvinyl chloride, copolymers of vinyl chloride and vinyl acetate and polyvinyl butyral, polyvinyl alcohol, polyvinyl acetal, ethylene-vinyl acetate copolymers, and ethylene-allyl copolymers such as ethylene-allyl alcohol copolymers, ethylene-allyl acetone copolymers, ethylene-allyl benzene copolymers ethylene-allyl ether copolymers, ethylene-acrylic copolymers and polyoxymethylene, polycondensation polymers, such as, polyesters, polyurethanes, polyamides and polycarbonates. The layer-forming polymers used on the supports for the transparent elements fused in the method of this invention and the supports are each well known to those skilled in the art, as are methods for forming the coated supports. Suitable polymers are film-forming polymers and include those described in U.S. Pat. No. 4,968,578, issued Nov. 6, 1990, which is hereby incorporated by reference herein. The polymers described in that patent for forming polymer surface layers on supports are film-forming addition or condensation polymers, which can be used as blends to provide the most desirable polymer surfaces. The preferred condensation polymers described in the aforementioned patent have average molecular weights in the range of about 20,000 to 80,000 while the preferred addition polymers have average molecular weights in the range of about 50,000 to 500,000. Specific classes of layer-forming (or film-forming polymers) described in U.S. Pat. No. 4,968,578 are polyesters, polystyrenes, polystyrene-acrylic, polymethyl methacrylate, polyvinyl acetate, polyolefins and copolymers such as poly(vinylethylene-co-acetate), polyethylene-co-acrylics, amorphous polypropylene and copolymers and graft copolymers of polypropylene. Particularly useful polymers are polyesters such as a copolyester of 50 mole percent terephthalic acid 50 mole percent neopentyl glycol and 50 mole percent diethylene glycol, a copolyester of 50 mole percent terephthalic acid, 90 mole percent neopentyl glycol and 10 mole percent diethylene glycol and mixtures of these copolymers.

Fusible toner particles used in this invention typically can have fusing temperatures of less than about 200° C., often less than about 100° C. They can readily be fused to transparent supports and have the capability of being

fused to paper sheets, even resin coated paper sheets without deformation (blistering) of the resin coating to form a low luster or non-glossy finish that has been found to be desirable in copies viewed by reflection. Of course, if the toner images are fused to supports which can withstand higher temperatures, toner particles of higher fusing temperatures can be used.

Numerous colorant materials selected from dyestuffs or pigments can be employed in the toner particles used in the invention. Such materials serve to color the toner and/or render it more visible. The colorants can, in principle, be selected from virtually any of the compounds mentioned in the Colour Index Volumes 1 and 2, Second Edition. Included among the vast number of useful colorants are those dyes and/or pigments that are typically employed as blue, green, red and yellow colorants used in electrostatographic toners to make color copies. Suitable colorants also include those typically employed in primary substrative cyan, magenta and yellow colored toners. Examples of useful colorants are Hansa Yellow G (C.I. 11680) CI Yellow 12, Ci Solvent Yellow 16, CI Disperse Yellow 33, Nigrosine Spirit soluble (C.I. 50415), Fuchsine N (C.I. 42510) C.I. Pigment Red 22, C.I. Solvent Red 19, C.I. Basic Blue 9 (C.I. 52015) and Pigment Blue 15. The amount of colorant added may vary over a wide range, for example, from about 1 to 20 percent of the weight of binder polymer used in the toner particles. Good results are obtained when the amount is from about 1 to 10 percent.

To utilize a binder polymer in an electrostatographic toner used in the practice of this invention, the polymer particles are mixed in any convenient manner with any other desired addenda, to form a free-flowing powder of toner particles containing the binder polymer. Useful toner particles can simply comprise the binder polymer and colorant but, it is often desirable to incorporate addenda such as waxes, release agents, charge control agents, and other toner addenda well known in the art.

Charge control agents suitable for use in toners are disclosed for example in U.S. Pat. Nos. 3,893,935; 4,079,014; 4,323,634 and British Patent Nos. 1,501,065 and 1,420,839. Charge control agents are generally employed in small quantities such as, about 0.1 to 3, weight percent, often about 0.2 to 1.5 weight percent, based on the weight of toner.

Toner images fused according to this invention can be formed from electrostatographic developers comprising toner particles that are mixed with a carrier vehicle. Carrier vehicles which can be used to form suitable developer compositions, can be selected from a variety of materials. Such materials include carrier core particles and core particles overcoated with a thin layer of film-forming resin. Examples of suitable resins are described in U.S. Pat. Nos. 3,547,822; 3,632,512; 3,795,618; 3,898,170; 4,545,060; 4,478,925; 4,076,857; and 3,970,571.

The carrier core particles can comprise conductive, non-conductive, magnetic, or non-magnetic materials. See, for example, U.S. Pat. Nos. 3,850,663 and 3,970,571. Especially useful in magnetic brush development schemes are iron particles such as porous iron particles having oxidized surfaces, steel particles, and other "hard" or "soft" ferromagnetic materials such as gamma ferric oxides or ferrites, such as ferrites of barium, strontium, lead, magnesium, or aluminum. See for example, U.S. Pat. Nos. 4,042,518; 4,478,925; and 4,546,060.

A typical developer composition containing toner particles and carrier vehicle generally comprises about 1 to 20 percent, by weight, of particulate toner particles and from 80 to 99 percent, by weight, carrier particles. Usually, the carrier particles are larger than the toner particles. Conventional carrier particles have a particle size on the order of about 20 to 1200 micrometers, generally about 30 to 300 micrometers. Alternatively, the toners can be used in a single component developer, i.e., with no carrier particles.

The toner and developer compositions described in the previous paragraphs can be used in a variety of ways to develop electrostatic charge patterns to provide the electrostatographic toner images fused by the method of this invention. Such developable charge patterns can be prepared by a number of means and be carried for example, on a light sensitive photoconductive element or a non-light-sensitive dielectric-surfaced element such as an insulator-coated conductive sheet. One suitable development technique involves cascading the developer composition across the electrostatic charge pattern, while another technique involves applying toner particles from a magnetic brush. This latter technique involves the use of a magnetically attractable carrier vehicle in forming the developer composition. After image-wise deposition of the toner particles to form an electrostatographic toner image, the image can be fixed or fused by the method of this invention to the support carrying the image which in this case, is a transparent support comprising a polymer layer. If desired, the unfused toner image can be transferred to a transparent support and then fused to form a permanent colored toner image thereon.

Typical toner particles generally have an average particle size in the range of about 0.1 to 100 micrometers, a size of about 8 to 15 micrometers being particularly useful in the practice of this invention to form high resolution images.

In the method of this invention the toner image is brought into pressure contact with the surface of the fusing member in the fusing zone. The temperature and pressure applied to fuse the toner particles causes the particles and the polymer layer bearing such particles to flow and form a toner image that does not exhibit the light scatter and internal reflections so detrimental to high color clarity. As a result, the fusing method of this invention provides transparencies having colored toner images on transparent supports which images exhibit exceptional color clarity. As known to those skilled in the art, color clarity can be defined as the ratio of specular to total transmitted light expressed in percent. Such color clarity can be conveniently determined by placing an image on a transparent support in an optical light path and separately measuring or reading the specular and totally transmitted light with a suitable device, e.g., a photometer.

Typical temperatures used in the fusing zone where the fusing member initially contacts the toner image are in the range of about 100° C. to 140° C., often 105° C. to 135° C. and preferably 115° C. to 130° C. The pressure used in the method of this invention in combination with the aforementioned fusing temperature when the transparent support bearing the unfused colored toner particles initially contacts the fusing member include those conventionally employed in contact fusing processes in the prior art. They are generally in the range of about 3 kg/cm<sup>2</sup> to 15 kg/cm<sup>2</sup> and often about 10 kg/cm<sup>2</sup>. As indicated in FIGS. 1 and 2, such pressure is

conveniently applied using a roll, although any suitable pressure means known to those skilled in the art could be used.

The fusing member employed in the practice of this invention can be in any physical form suitable for applying heat in face-to-face relationship with the unfused toner image and maintaining such relationship through the cooling zone. Examples are the continuous belt 4 indicated in FIG. 1 or the roll 10 indicated in FIG. 2, although the fusing member can also be in the form of a plate. A continuous belt is preferred because this provides a straight, flat fusing path which reduces curl problems that can be introduced by a roll. When a continuous belt is employed, the belt must be reasonably flexible and also heat resistant; it is preferably made with a material such as stainless steel or polyester which meet such criteria. The outer surface of the fusing member which contacts the toner image can comprise a wide variety of materials known in the prior art to be suitable for use in such fusing surfaces, including aluminum, steel, various alloys as well as polymeric materials such as thermoset resins. Fusing members with fluorocelastomer surfaces can improve the release characteristics of the fuser member. Also release agents, for example, polymeric release oils such as polydiorganosiloxane release oils can be used. However, such additional release agents are frequently unnecessary in the practice of this invention because the toner image and polymer layer on the support are cooled in the cooling zone to a level where they readily release from the fusing member without toner image or polymer offset i.e. there is no transfer of toner image or polymer to the surface of the fusing member. The toner image to be fused normally moves through the fusing zone at a velocity of at least about 2.5 cm/sec., typically about 2.5 to 10 cm/sec. The velocity is generally kept constant as the element bearing the toner image moves through the cooling and release zones.

In the cooling zone, cooling of the fused toner image and polymer layer on the support is controlled so that they can be released at a temperature where no offset occurs. The temperature of the fused image and polymer layer are generally reduced at least about 40° C., often about 65° to 90° C. in the cooling zone. As previously indicated herein, cooling can be conveniently controlled simply by adjusting the velocity of the fusing member, for example, the velocity of a continuous belt or roll while cooling air is impinged upon the belt, or upon the element, as in FIG. 2, although other cooling means such as a chill roll or plate could be used in place of air impingement. When a continuous belt is used as the fusing member, it usually is not necessary to press the element against the fusing member to maintain contact between the fusing member and the toner image because the toner image and polymer layer are heated in the fusing zone to a point where their surfaces act as an adhesive which temporarily bonds to the fusing member as the element moves through the cooling zone.

In the release zone the fused toner image is separated from the fusing member. Such release is not effected until the fusing member is cooled to a temperature where no toner image or polymer offset occurs. Such temperature is typically no more than about 75° C. and is normally in the range of about 30° C. to 60° C. The specific temperature used to achieve such separation will vary considerably as it depends upon the specific viscoelastic properties of the toner image and the polymer layer bearing such image. The release temperature

chosen is one at which the toner image and polymer layer exhibit elastic flow characteristic and adhere to the support and exhibit sufficient cohesiveness so they will not offset onto the fuser member at the particular temperature used.

The elements fused in the method of this invention comprises a transparent support. A wide variety of such supports are known and commonly employed in the electrostatographic art. They include, for example, those supports used in the manufacture of photographic films including cellulose esters such as cellulose triacetate, cellulose acetate propionate or cellulose acetate butyrate, polyesters such as poly(ethylene terephthalate), polyamides, polycarbonates, polyimides, polyolefins, poly(vinyl acetals), polyesters and poly sulfonamides. Polyester film supports, and especially poly(ethylene terephthalate) are preferred because of their excellent dimensional stability characteristics. When such a polyester is used as the support material, a subbing layer is advantageously employed to improve the bonding of the polymer layer bearing the toner image to the support. Useful subbing compositions for this purpose are well known in the photographic art and include, for example, polymers of vinylidene chloride such as vinylidene chloride/acrylonitrile/acrylic acid terpolymers or vinylidene chloride/methyl acrylate/itaconic acid terpolymers.

The following preparation and fusing techniques and examples are presented to further illustrate this invention.

In some of the preparations and examples polymer names contain an indication of the molar or weight ratios of the various units in the polymer, as specified. In some of the preparations and examples (as indicated therein), the relative concentrations of units are expressed as ratios or amounts of the monomers used to prepare the polymer.

#### Developer Formulation, Imaging and Fusing

Toner particles employed to form the toner images in the following examples were formulated from 100 parts binder polymer, 0-20 parts colorant, 0-20 parts addenda and 0-2 parts of charge agent per 100 parts bonder polymer. The mixtures were melt-compounded at temperatures in the range of 110° to 150° C. on a 2-roll rubber mill, the mass cooled to room temperature, and coarse ground and fluid energy-milled to produce toner particles having a particle size in the range of about 8 to 15 micrometers.

The toner particles were then mixed with carrier particles in a closed container on a 2-roll mill for 30 seconds to form a triboelectrically-charged 2-component dry electrostatographic developer comprising about 13 weight percent toner particles. The carrier particles employed were strontium ferrite particles coated with a thin poly(vinylidene fluoride) film.

The electrostatographic developer was used to develop a toner image on transparent poly(ethylene terephthalate) film 76 micrometers thick, subbed with a terpolymer of acrylonitrile, vinylidene chloride and acrylic acid, and coated with a layer 10 micrometers thick of a polyester blend, (60/40, wgt percent, having a T<sub>g</sub> of 50° C. and a weight average molecular weight of about 30,000) of a condensation polymer of 50 mole percent terephthalic acid reacted with a 50/50 mole percent mixture of neopentyl glycol and diethylene glycol, and 50 mole percent of terephthalic acid reacted with a 90/10 mole percent mixture of neopentyl glycol

and diethylene glycol. The blend had a loss tangent of 2.1 determined for a storage modulus, G', of 10<sup>5</sup> dynes/cm<sup>3</sup> (G' of 1.15 × 10<sup>2</sup> dynes/cm<sup>2</sup>, G'' of 4.86 × 10<sup>3</sup> dynes/cm<sup>2</sup> and a melt viscosity of 4.86 × 10<sup>3</sup> poise measured at a temperature of 150° C. and 1 rad/sec.) all measured using a Rheometric Model RDA 700 rheometer (commercially available from Rheometrics, Inc., Piscataway, N.J.) using parallel plates in a sinusoidal shear mode.

Biased development was carried out in an electrophotographic copying apparatus having an organic photoconductor film, a magnetic brush developing station and a biased roll transfer station for transferring the toner image from the photoconductor film to the poly(ethylene terephthalate) film support. The toner image comprised a line copy toner image developed with toner particles having a loss tangent of up to 1.5.

The toner image was fused using a fusing device of the type illustrated in FIG. 1 in which the fusing member was a continuous highly polished smooth steel belt. The fusing conditions used were as follows:

|                             |                         |
|-----------------------------|-------------------------|
| Belt Velocity               | 6.5 cm/sec.             |
| Fusing Temperature          | 105°-130° C.            |
| Pressure                    | 3-15 kg/cm <sup>2</sup> |
| Nip Width                   | 0.4-0.6 cm              |
| Cooling Air Temperature     | 20°-25°                 |
| Release Temperature at Roll | 40°-65° C.              |

#### EXAMPLE 1

The fusing method of this invention is effective to provide a projection viewable transparency having excellent color clarity. To illustrate, a developer composition comprising the following toner was prepared as described previously in the Developer Formulation, Imaging and Fusing section.

Toner particles were formulated from 100 parts of a binder polymer comprising 90 percent, by weight poly(styrene-co-n-butylacrylate)[77/23 weight percent] cross-linked with 0.4 parts per hundred divinylbenzene, having a T<sub>g</sub> of 65° C., a weight-average molecular weight ( $\bar{M}_w$ ) of 275,000 and a number-average molecular weight ( $\bar{M}_n$ ) of 31,000 and 10 percent, by weight, of polystyrene having a T<sub>g</sub> of 102° C. a ( $\bar{M}_w$ ) of 285,000 and a ( $\bar{M}_n$ ) of 102,000, 6 parts of a cyan colorant and 1 part of a quaternary ammonium charge agent. The pulverized toner particles were classified to provide cyan toner particles having a particle size of 10 to 12 micrometers and a loss tangent of 0.7 determined for a storage modulus, G', of 10<sup>5</sup> dynes/cm<sup>3</sup> (G' of 2.33 × 10<sup>5</sup> dynes/cm<sup>2</sup>, G'' of 1.29 × 10<sup>5</sup> dynes/cm<sup>2</sup> and melt viscosity of 2.66 × 10<sup>5</sup> poise measured at a temperature of 150° C. and 1 rad/sec.) all measured using a Rheometrics Model RDA 700 rheometer (commercially available from Rheometrics, Inc., Piscataway, N.J.) using parallel plates in a sinusoidal shear mode. This Toner I was used to develop the a copy image, as previously described in the Developer Formulations, Imaging and Fusing section.

Upon projection in an overhead projector the cyan line copy image showed high color density and saturation comparable to that of the original image. The color clarity for the image, determined as described previously herein was approximately 90 percent. In comparison, the same image developed and fused on the poly(ethylene terephthalate) transparent support but with-

out the layer formed from the polyester blend, had a clarity of only 75 percent.

#### EXAMPLE 2

The procedure of Example 1 was repeated except that the following toner was substituted for the toner used in that example.

Toner particles were formulated from 100 parts of a binder polymer comprising 90 percent, by weight poly(styrene-co-n-butylacrylate)[77/23 weight percent], having a  $T_g$  of 68° C., a weight-average molecular weight ( $M_w$ ) of 47,000 and a number-average molecular weight ( $M_n$ ) of 23,000, and 10 percent, by weight, of a styrene-alkylene block copolymer (sold by Shell Chemical Co. under the designation "Kraton 1652") having a  $T_g$  of 90° C., 6 parts of a yellow colorant and 1 part of a quaternary ammonium charge agent. The pulverized toner particles were classified to provide yellow toner particles having a particle size of 8-10 micrometers and a loss tangent of 0.5 determined for a storage modulus,  $G'$ , of  $10^5$  dynes/cm<sup>3</sup> ( $G'$  of  $2.10 \times 10^5$  dynes/cm<sup>2</sup>,  $G''$  of  $1.26 \times 10^5$  dynes/cm<sup>2</sup> and melt viscosity of  $2.40 \times 10^5$  poise measured at a temperature of 150° C. and 1 rad/sec.) measured as described in Example 1. This toner was used to develop the line copy image as described in Example 1.

The color clarity for the image, determined as in Example 1, was approximately 85 percent while the color clarity of the fused toner image on the poly(ethylene) terephthalate) support without the layer of the 30 polyester was only 70 percent.

#### EXAMPLE 3

The procedure of Example 1 was repeated except that the polyester blend coated on the poly(ethylene 35 therphthalate film was replaced with a coating of poly-(styrene-co-n-butyl acrylate) [70/30 weight percent] having a  $T_g$  of 52° C., a  $M_w$  of 100,000 and a number average molecular weight of 30,000, and a loss tangent of 1.7 determined for a storage modulus,  $G'$ , of  $10^5$  40 dynes/cm<sup>3</sup> ( $G'$  of  $1.05 \times 10^3$ ,  $G''$  of  $7.54 \times 10^3$  and melt viscosity of  $7.61 \times 10^3$  poise measured at a temperature of 150° C. and 1 rad/sec.), determined as in Example 1. The color clarity of the fused line copy transparency 45 was 80 percent.

#### EXAMPLE 4

The procedure of Example 3 was repeated except that the following toner was substituted for the toner used in that example.

Toner particles were formulated from 100 parts of a binder polymer comprising poly(styrene-co-n-butylacrylate)[77/33 weight percent] crosslinked with 0.4 parts per hundred divinylbenzene, having a  $T_g$  of 65° C., a weight-average molecular weight ( $M_w$ ) of 275,000, 55 and a number-average molecular weight ( $M_n$ ) of 31,000, 6 parts of a blue colorant and 1 part of a quaternary ammonium charge agent. The pulverized toner particles were classified to provide blue toner particles having a particle size of 6-8 micrometers and loss tangent of 60 0.8 determined for a storage modulus,  $G'$ , of  $10^5$  dynes/cm<sup>3</sup> ( $G'$  of  $1.24 \times 10^5$  dynes/cm<sup>2</sup>,  $G''$  of  $8.54 \times 10^4$  dynes/cm<sup>2</sup> and melt viscosity of  $1.51 \times 10^5$  poise measured at a temperature of 150° C. and 1 rad/sec.), measured as described in Example 1. This toner was used to 65 develop the line copy image as described in Example 1.

The color clarity of the fused blue line copy transparency was 75 percent.

#### EXAMPLE 5

The procedure of Example 1 was repeated except that the following toner was used in place of the toner in that example.

Toner particles were formulated from 100 parts of a binder polymer comprising poly(styrene-co-n-butylacrylate)[80/20 weight percent] crosslinked with 1.3 parts per hundred divinylbenzene, having a  $T_g$  of 65° C., 10 a weight-average molecular weight ( $M_w$ ) of 410,000 and a number average molecular weight ( $M_n$ ) of 10,000, 6 parts of a yellow colorant and 1 part of a quaternary ammonium charge agent. The pulverized toner particles were classified to provide yellow toner particles having a particle size of 6-8 micrometers and a loss tangent of 1.2 determined for a storage modulus,  $G'$ , of  $10^5$  dynes/cm<sup>3</sup> ( $G'$  of  $4.98 \times 10^3$  dynes/cm<sup>2</sup>,  $G''$  of  $1.01 \times 10^4$  dynes/cm<sup>2</sup> melt viscosity of  $1.12 \times 10^4$  poise measured at a temperature of 150° C. and 1 rad/sec.) measured as described in Example 1. This toner was used to develop the line copy image as described in Example 1.

The color clarity of the fused line copy transparency determined as in Example 1, was 78 percent.

It is evident from the foregoing specification, and Particularly the Examples, that the fusing method of this invention makes it possible to obtain projection viewable transparencies comprising toner images of very high color clarity. Such color transparencies faithfully reproduce the color of an original image and exhibits excellent color saturation.

The invention has been described in detail with particular reference to certain preferred embodiments thereof, but it should be appreciated that variations in modification can be effected within the spirit and scope of the invention.

We claim:

1. A fusing method for making a transparency capable of projecting an electrostatographic colored toner image that exhibits excellent color clarity, which method comprises:
  - a. providing a transparent element having a transparent support comprising a polymer layer bearing an image in colored toner particles that exhibit a loss tangent ( $\tan \delta$ ) up to about 1.5 upon fusing the image with heat and pressure, the polymer forming such layer having a greater loss tangent ( $\tan \delta$ ) than the toner particles upon such fusing;
  - b. passing the element successively through a fusing zone, a cooling zone and a release zone;
  - c. within the fusing zone, bringing the image and polymer layer into pressure contact with a surface of a fusing member at a temperature that fuses the image to the support and causes the polymer layer to flow;
  - d. maintaining contact between the fused image and the fusing member within the cooling zone while reducing the temperature of the fusing member;
  - e. separating the fused image from the fusing member within the release zone at a temperature where the image and the polymer layer do not offset.
2. The method of claim 1, wherein the loss tangent of the toner particles is in the range of about 0.5 to 1.5.
3. The method of claim 2, wherein the toner image is a yellow toner image.
4. The method of claim 1, wherein the toner image comprises a polyester binder.

5. The method of claim 1, wherein the toner image comprises a styrene-acrylic copolymer binder.
6. The method of claim 1, wherein the fusing member is a continuous belt.
7. The method of claim 3, wherein the fusing member is a continuous belt.
8. The method of claim 7 wherein the temperature of the fusing member is less than about 140° C.

9. The method of claim 8, wherein the particle size of the toner particles is in the range of about 8 to 15 micrometers.
  10. The method of claim 1, wherein the polymer forming the layer on the support is a polyester.
  11. The method of claim 10, wherein the polyester is a copolyester of terephthalic acid with a mixture of neopentyl glycol and diethylene glycol.
- \* \* \* \* \*

10

15

20

25

30

35

40

45

50

55

60

65